

## UNITED STATES PATENT OFFICE

2,345,632

## POLYAMIDES

Edwin A. Robinson, Chatham, and Maurice J. Kelley, Newark, N. J., assignors to National Oil Products Company, Harrison, N. J., a corporation of New Jersey

No Drawing. Application May 20, 1939.  
Serial No. 274,808

13 Claims. (CL 260—404.5)

This invention relates to textile lubricants and softeners, more particularly to textile lubricants and softeners comprising mixed fatty polyamides.

It has been proposed to use higher fatty amides, such as oleic acid amide, oleic acid methyl amide and oleic acid ethylene diamide as softeners and lubricants for textile materials. Such amides are ordinarily prepared by reacting a fatty acid or fatty ester with a mono- or poly-amine. The reaction of monoamines with higher fatty acids or fatty esters yields products which are not readily dispersible in water, and since these products contain no residual amino group, they may not be solubilized to any substantial extent by treatment with acids. Hence these products may not be advantageously applied to textile material. It has been proposed, therefore, to react polyamines with higher fatty acids or fatty esters to produce amides having free amino groups capable of reacting with weak acids so as to solubilize the products and render them readily dispersible or soluble in water. However, the monoamides formed from such polyamines by reaction thereof with higher fatty acids or fatty esters cause yellowing of textile material upon application thereto, and hence are highly unsuitable for use as textile lubricants and softeners. On the other hand, polyamides formed by the reaction of higher fatty acids or fatty esters with polyamines are much less desirable as softeners and lubricants than the corresponding monoamides because of their relatively poor softening and lubricating properties.

It has also been proposed to prepare textile lubricants and softeners by reacting unsymmetrical dialkyl ethylene diamine with higher fatty acids such as oleic acid. Such unsymmetrical dialkyl amines are, however, relatively expensive and difficult to obtain, and hence, while the amides thereof have been used to some extent as textile lubricants and softeners, there is a great demand in the textile industry for cheaper products which may be used in place of these amides.

It is the object of this invention to provide inexpensive and highly effective textile lubricants and softeners.

It is a further object of this invention to pro-

vide a process for the preparation of textile lubricants and softeners from polyamines.

We have now found that polyamides having the general formula  $R_1CO-NR_3-X-COR_2$  in which  $R_1$  stands for an alkyl radical containing from 7 to 21 carbon atoms,  $R_2$  stands for an alkyl radical containing from 1 to 4 carbon atoms,  $R_3$  stands for hydrogen or an acyl group containing from 2 to 5 carbon atoms and  $X$  stands for the grouping  $(-CR_4R_5-CR_4R_5-NR_3)_n$ , wherein  $R_4$  and  $R_5$  stand for hydrogen or alkyl radicals, and  $n$  is a whole number, may be applied to textile materials so as to impart thereto excellent softness, drape and pliability without causing yellowing of the material. The preferred polyamides of our invention may be prepared in a simple and inexpensive manner by reacting a readily available polyamine such as ethylene diamine, diethylene triamine, triethylene tetramine, etc., with a fatty acid containing from 8 to 22 carbon atoms or an ester thereof, and with a short chain fatty acid containing from 2 to 5 carbon atoms or an ester, anhydride or acid halide thereof. Preferably, the polyamides of our invention contain one secondary amino group so that they may be treated with weak acids for the production of solubilized modifications of the polyamides. We have found that the presence of substantially more than one secondary amino group in the polyamides of our invention tends to cause objectionable yellowing of the textile material to which the polyamide is applied; hence, if polyamines containing more than 2 nitrogen atoms, e. g., triethylene tetramine or tetraethylene pentamine, are employed to prepare the products of our invention, preferably sufficient amounts of the short chain fatty acid are employed so as to acylate all but one of the secondary amino groups.

40 The products of our invention are preferably prepared by reacting a polyamine with a higher fatty acid containing from 8 to 22 carbon atoms, preferably from 12 to 18 carbon atoms, or an ester thereof so as to form a monoamide, and then reacting the monoamide with suitable amounts of an acid containing from 2 to 5 carbon atoms. However, when employing diamines or triamines in the practice of our invention, the preparation of the amides may be carried out by first reacting the polyamine with the short

chain acid and then treating the product with the long chain fatty acid. Any polyamine may be used in the practice of our invention; thus, for example, polyamines such as ethylene diamine, diethylene triamine, triethylene tetraamine, tetra ethylene pentamine and hydroxyethyl ethylene diamine may be employed. We prefer to use diethylene triamine since we have found that amides prepared from this polyamine in accordance with our invention are highly effective textile lubricants and softeners, do not yellow textile material to which they are applied and may be readily solubilized by treatment with weak acids; furthermore, diethylene triamine is relatively inexpensive and readily available.

The long chain fatty acid compound reacted with the polyamine in accordance with our invention may be any of the fatty acids containing from 8 to 22 carbon atoms, preferably from 12 to 18 carbon atoms, or the esters thereof; the following higher fatty acids may be mentioned by way of examples: caprylic acid, nonylic acid, capric acid, undecylic acid, lauric acid, myristic acid, palmitic acid, stearic acid, behenic acid, oleic acid, ricinoleic acid, mixtures of these acids, etc. In place of the higher fatty acids, derivatives thereof such as glycerides and other esters, may be employed. Actually, we prefer to use glycerides of the fatty acids since products are obtained having superior softening properties to those resulting from the reaction of the polyamines with the free fatty acids. Products particularly suitable as textile lubricants and softeners are obtained by employing coconut oil to react with the polyamines in accordance with our invention, since these products are dispersible in water without further solubilizing treatment and possess excellent lubricating and softening properties. As examples of other glycerides that may be employed in place of the long chain fatty acids, there may be mentioned teaseed oil, castor oil, hydrogenated castor oil, etc.

The short chain acids employed in accordance with our invention contain from 2 to 5 carbon atoms; thus, for example, acetic acid, lactic acid, propionic acid, butyric acid and valeric acid may be employed; derivatives thereof such as esters, acid halides and anhydrides may be employed in accordance with procedures well known to the art. We prefer to use acetic acid or acetic anhydride in the preparation of our novel products because of their ready availability and the excellent softening properties of the amides prepared from these compounds.

In carrying out the reaction in accordance with our preferred method, approximately equimolecular quantities of a polyamine and a fatty acid containing from 8 to 22 carbon atoms are mixed; if a glyceride of a fatty acid is employed, e. g., coconut oil, approximately  $\frac{1}{3}$  mol of the glyceride per mol of polyamine is used. The compounds are then permitted to react at a temperature sufficiently high to cause the formation of the monoamide; this temperature may vary from about 120° C. to about 200° C., but preferably is between about 150° C. and about 170° C. The time of this reaction may vary widely depending somewhat upon the particular reactants and somewhat upon the temperature; generally, 8 hours or more are required. The pressure under which the reaction is carried out is preferably atmospheric; however, pressures above or below atmospheric may be employed. The product of the reaction is then mixed with a suitable quantity of a short chain fatty acid containing from 2

to 5 carbon atoms; as above mentioned, anhydrides, esters or acid halides of these acids may also be employed. The amount of short chain acid compound employed depends to some extent upon the number of amino groups to be acylated and the nature of the compound used. Thus in the case of diethylene triamine, we prefer to employ about 1 mol of a short chain fatty acid per mol of diethylene triamine; however, in the case of triethylene tetraamine, where it is desired to acylate not only the  $-\text{NH}_2$  group but also one of the secondary amino groups, approximately 2 mols of the short chain acid per mol of the polyamine may be employed. It is to be understood that if derivatives of the short chain acid are reacted with the monoamide, the amounts thereof will be adjusted accordingly; for example, approximately one-half mol of acetic anhydride is used where one mol of acetic acid is required. If desired, sufficient amounts of the short chain acid may be used so as to form two amido groups on the free  $-\text{NH}_2$  group; the  $-\text{NH}-$  group adjacent the long chain fatty group may also be acylated. Generally, it may be said that the number of mols of short chain fatty acid employed per mol of polyamine will be equivalent to the number of groups to be acylated in accordance with our invention. The conditions under which this reaction is carried out may vary widely, but we have found that the constituents may be reacted at atmospheric pressure and at a temperature of about 135° C. for about 3 to 5 hours, the mixture then raised to between about 150° C. and about 170° C., and the reaction continued for about 5 to about 8 additional hours with excellent results. However, it is to be understood that these conditions may be varied somewhat without affecting the course of the reaction, e. g., pressures above or below atmospheric may be used, the temperatures may vary widely so long as they are sufficiently high to effect acylation, and the time of reaction may differ from the time above set forth.

The products of our invention may be liquids or solids, but generally they are solids. The majority of these products are relatively insoluble in water; however, products somewhat soluble or dispersible in water may be obtained. As above mentioned, the coconut oil products are generally dispersible in water. The preferred products of our invention contain a free secondary amino group so that they may be treated with weak acids such as acetic acid or lactic acid to solubilize the amide and render them more soluble or dispersible in water. The solubilizing treatment is preferably carried out by mixing a dilute solution of the weak acid with the molten polyamide, stirring the mixture until it is homogeneous, then permitting the mixture to cool and recovering the solubilized amide. Our novel products may be marketed as such or in the form of an aqueous solution, dispersion or paste thereof. They may be applied to textile material by any of the well known methods, e. g., in the form of a dilute solution thereof, and in every case impart excellent softness, drape, flexibility and handle to the textile material.

The following examples are illustrative of our invention. Amounts are given in parts by weight.

#### Example I

300 parts of coconut oil and 143 parts of diethylene triamine were mixed and the mixture agitated at temperatures between 150° C. and 170° C. for 8 hours. 312 parts of the reaction product were then mixed with 50 parts of acetic

anhydride, the mixture agitated at a temperature of 135° C. for 4½ hours, the temperature then raised to 160° C. and the reaction continued for 3 more hours. The product thus obtained was a solid relatively dispersible in water.

*Example II*

587 parts of coconut oil and 277 parts of diethylene triamine were mixed in an open kettle and agitated at a temperature of 150° C. for 8 hours. The mixture was then permitted to cool to just above the melting point of the reaction product (about 50° C.). 136 parts of acetic anhydride were added to the molten mass, and the mixture agitated at a temperature of 135° C. for 5 hours, the temperature then raised to 150° C. and the reaction continued for 3 more hours. The product thus obtained was a light tan solid relatively dispersible in water. This product was then melted, mixed with approximately 5400 parts of a hot 3% solution of acetic acid, the mixture stirred at a temperature above the melting point of the amide until homogeneous, then cooled and a product soluble in water recovered.

*Example III*

190 parts of tetraethylene pentamine and 230 parts of coconut oil were mixed in an open kettle and agitated at a temperature between 150° C. and 170° C. for 8 hours. 153 parts of acetic anhydride were then added to the reaction product and the mixture agitated at a temperature of 135° C. for 3 hours, the temperature was then raised to between 150° C. and 170° C. and the reaction continued for 5 more hours. The product thus obtained was relatively soluble in water. The product was then melted, mixed with about 2000 parts of a hot 3% solution of acetic acid, the mixture stirred at a temperature above the melting point of the amide until homogeneous, then cooled and a product soluble in water recovered.

*Example IV*

60 parts of ethylene diamine and 230 parts of coconut oil were mixed in an open kettle and agitated at a temperature between 150° C. and 170° C. for 8 hours. 50 parts of acetic anhydride were then added to the reaction product and the mixture agitated at a temperature of 135° C. for 3 hours, the temperature raised to between 150° C. and 170° C. and the reaction continued for an additional 5 hours. A solid product relatively insoluble in water was thereby obtained.

*Example V*

679 parts of coconut oil and 321 parts of hydroxy ethyl ethylene diamine were mixed in an open kettle and agitated at temperatures between 150° C. and 170° C. for 8 hours. 260 parts of the reaction product were then mixed with 47 parts of acetic anhydride, the mixture agitated at a temperature of 135° C. for 5 hours, the temperature then raised to between 150° C. and 170° C. and the reaction continued for 5 more hours. The product was a clear, reddish amber liquid dispersible in water.

*Example VI*

186 parts of teaseed oil and 65 parts of diethylene triamine were mixed in an open kettle and agitated at temperatures between 150° C. and 170° C. for 8 hours. 32 parts of acetic anhydride were then added to the reaction product and the mixture agitated at a temperature of 135° C. for 3 hours, the temperature raised to

between 150° C. and 170° C. and the reaction continued for 7 more hours. The product was a viscous brown liquid relatively insoluble in water. This product was melted, mixed with about 1400 parts of a hot 3% acetic acid solution, the mixture stirred at a temperature above the melting point of the amide until homogeneous, then cooled and a product soluble in water recovered.

*Example VII*

280 parts of oleic acid and 103 parts of diethylene triamine were mixed in an open kettle and the mixture agitated at temperatures between 150° C. and 170° C. for about 12 hours. 51 parts of acetic anhydride were then added to the reaction product and the mixture agitated at a temperature of 135° C. for 3 hours, the temperature raised to between 150° C. and 170° C. and the reaction continued for 7 more hours. The product was a viscous brown liquid relatively insoluble in water. This product was melted, mixed with about 2000 parts of a hot 3% acetic acid solution, the mixture stirred at a temperature above the melting point of the amide until homogeneous, then cooled and a product soluble in water recovered.

*Example VIII*

256 parts of palmitic acid and 103 parts of diethylene triamine were mixed in an open kettle and the mixture agitated at temperatures between 150° C. and 170° C. for 12 hours. 51 parts of acetic anhydride were then added to the reaction product and the mixture agitated at a temperature of 135° C. for 3 hours, the temperature raised to between 150° C. and 170° C. and the reaction continued for 7 more hours. The product was insoluble in water. It was melted, mixed with about 2000 parts of a hot 3% acetic acid solution, the mixture stirred at a temperature above the melting point of the amide until homogeneous, then cooled and a product soluble in water recovered.

*Example IX*

200 parts of lauric acid and 103 parts of diethylene triamine were mixed in an open kettle and the mixture agitated at temperatures between 150° C. and 170° C. for 12 hours. 51 parts of acetic anhydride were then added to the reaction product and the mixture agitated at a temperature of 135° C. for 3 hours, the temperature raised to between 150° C. and 170° C. and the reaction continued for 7 more hours. The product was insoluble in water. It was melted, mixed with about 2000 parts of a hot 3% acetic acid solution, the mixture stirred at a temperature above the melting point of the amide until homogeneous, then cooled and a product soluble in water recovered.

*Example X*

284 parts of stearic acid and 103 parts of diethylene triamine were mixed in an open kettle and the mixture agitated at temperatures between 150° C. and 170° C. for 12 hours. 51 parts of acetic anhydride were then added to the reaction product and the mixture agitated at a temperature of 135° C. for 3 hours, the temperature raised to between 150° C. and 170° C. and the reaction continued for 5 more hours. The product thus obtained was insoluble in water. It was melted, mixed with 2000 parts of a hot 3% acetic acid solution, the mixture stirred at a temperature above the melting point of the amide until

homogeneous and a product soluble in water recovered.

In place of the acetic anhydride, 90 parts of lactic acid may be added; in place of the hot acetic acid solution, 3000 parts of a hot 3% lactic acid solution may be employed.

The polyamides obtained as above described have been found to be excellent textile lubricants and softeners. They impart to the textile material treated therewith excellent softness, drape, flexibility and handle, but do not cause any appreciable yellowing of the material even after prolonged contact therewith. The products of our invention have been found to give a softer finish when applied to textiles than the fatty amides of unsymmetrical dialkyl diamines hereinabove referred to; hence, smaller amounts of our products may be used to soften textiles than are necessary when the latter amides are employed. Furthermore, our products cause less discoloration of the textile material to which they are applied than do the amides of unsymmetrical dialkyl diamines. In addition, the products of our invention are much easier to use than the amides of the unsymmetrical dialkyl diamines since they may be dispersed or dissolved in water with great ease, in contrast to the difficulties encountered in dispersing or dissolving the latter amides. As above pointed out, our novel products may be prepared from readily available and inexpensive amines, and hence are much cheaper than the fatty amides of the unsymmetrical dialkyl diamines. Therefore, in view of the above, it is evident that the products of our invention display a marked superiority over lubricants and softeners heretofore used in the textile industry, and hence will be of great value to textile manufacturers.

In addition to their use as textile lubricants and softeners, the products of our invention may be employed for a wide variety of other purposes; for example, they may be used as lubricants and softeners for other fibrous material such as leather, paper, etc. They may be added to viscose spinning baths to prevent clogging of the spinnerets, and may be used as defoaming agents, assistants in dyeing, printing and otherwise treating textiles and the like, and for the preparation of detergents and wetting, dispersing and emulsifying agents.

Since certain changes may be made in the above products and different embodiments of the invention may be made without departing from the scope thereof, it is intended that all matter contained in the above description shall be interpreted as illustrative and not in a limiting sense.

Having described our invention, what we claim as new and desire to secure by Letters Patent, is:

1. A compound selected from the group consisting of polyamides having the general formula  $R_1CO-NR_3-X-COR_2$  in which  $R_1CO$  stands for a fatty acyl radicle containing from 8 to 22 carbon atoms,  $COR_2$  stands for a fatty acyl radicle containing from 2 to 5 carbon atoms,  $R_3$  stands for a radical selected from the group consisting of hydrogen and acyl radicals containing from 2 to 5 carbon atoms and  $X$  stands for the grouping  $(-CR_4R_5-CR_4R_5-NR_3)_n$  in which  $R_4$  and  $R_5$  stand for radicals selected from the group consisting of hydrogen and alkyl radicals and  $n$  is a whole number greater than one, and salts of said polyamides with weak acids.

2. Polyamides having the general formula  $R_1CO-NR_3-X-COR_2$  in which  $R_1CO$  stands for

a fatty acyl radicle containing from 8 to 22 carbon atoms,  $COR_2$  stands for a fatty acyl radicle containing from 2 to 5 carbon atoms,  $R_3$  stands for a radical selected from the group consisting of hydrogen and acyl radicals containing from 2 to 5 carbon atoms, and  $X$  stands for the grouping  $(-CR_4R_5-CR_4R_5-NR_3)_n$  in which  $R_4$  and  $R_5$  stand for radicals selected from the group consisting of hydrogen and alkyl radicals, and  $n$  is a whole number greater than one.

3. Polyamides having the general formula  $R_1CO-NR_3-X-COR_2$  in which  $R_1CO$  stands for a fatty acyl radicle containing from 12 to 18 carbon atoms,  $COR_2$  stands for a fatty acyl radicle containing from 2 to 5 carbon atoms,  $R_3$  stands for a radical selected from the group consisting of hydrogen and acyl radicals containing from 2 to 5 carbon atoms, and  $X$  stands for the grouping  $(-CR_4R_5-CR_4R_5-NR_3)_n$  in which  $R_4$  and  $R_5$  stand for radicals selected from the group consisting of hydrogen and alkyl radicals, and  $n$  is a whole number greater than one.

4. Polyamides having the general formula  $R_1CO-NR_3-X-COR_2$  in which  $R_1CO$  stands for a fatty acyl radicle containing from 8 to 22 carbon atoms,  $COR_2$  stands for a fatty acyl radicle containing from 2 to 5 carbon atoms,  $R_3$  stands for a radical selected from the group consisting of hydrogen and acyl radicals containing from 2 to 5 carbon atoms, and  $X$  stands for the grouping

$-CR_4R_5-CR_4R_5-NH-(CR_4R_5-CR_4R_5-NR_3)_n$

in which  $R_4$  and  $R_5$  stand for radicals selected from the group consisting of hydrogen and alkyl groups, and  $n$  is a whole number.

5. Weak acid salts of and polyamides having the general formula  $R_1CO-NR_3-X-COR_2$  in which  $R_1CO$  stands for a fatty acyl radicle containing from 8 to 22 carbon atoms,  $COR_2$  stands for a fatty acyl radicle containing from 2 to 5 carbon atoms,  $R_3$  stands for a radical selected from the group consisting of hydrogen and acyl radicals containing from 2 to 5 carbon atoms, and  $X$  stands for the grouping

$-CR_4R_5-CR_4R_5-NH-(CR_4R_5-CR_4R_5-NR_3)_n$

in which  $R_4$  and  $R_5$  stand for radicals selected from the group consisting of hydrogen and alkyl radicals, and  $n$  is a whole number.

6. Polyamides having the general formula  $R_1CO-NH-X-COR_2$  in which  $R_1$  stands for the mixture of the alkyl radicals of coconut fatty acids,  $COR_2$  stands for a fatty acyl radicle containing from 2 to 5 carbon atoms, and  $X$  stands for the grouping  $(CH_2-CH_2-NR_3)_n$  in which  $R_3$  stands for a radical selected from the group consisting of hydrogen and acyl radicals containing from 2 to 5 carbon atoms, and  $n$  is a whole number greater than one.

7. Polyamides having the general formula  $R_1CONH-CH_2CH_2NHCH_2CH_2NHCO$  in which  $R_1$  stands for the mixture of the alkyl radicals of coconut fatty acids and  $COR_2$  stands for a fatty acyl radicle containing from 2 to 5 carbon atoms.

8. A polyamide having the general formula  $R_1CONHCH_2CH_2NHCH_2CH_2NHCOCH_3$  in which  $R_1$  stands for the mixture of the alkyl radicals of coconut fatty acids.

9. An acetic acid salt of a polyamide having the general formula

$R_1CONHCH_2CH_2NHCH_2CH_2NHCOCH_3$

in which  $R_1$  stands for the mixture of the alkyl radicals of coconut fatty acids.

10. An acetic acid salt of a polyamide having the general formula



11. A process for the preparation of polyamides which comprises condensing a polyamine with a compound selected from the group consisting of fatty acids containing from 8 to 22 carbon atoms and the esters thereof, and with a compound selected from the group consisting of fatty acids containing from 2 to 5 carbon atoms and the esters, anhydrides and acid halides thereof.

12. A process for the preparation of polyamides which comprises condensing diethylene triamine

and coconut oil to form a monoamide, and then reacting the monoamide with acetic anhydride so as to form a diamide.

13. Polyamides having the general formula



in which  $\text{R}_1\text{CO}$  stands for a fatty acyl radicle containing from 8 to 22 carbon atoms,  $\text{COR}_2$  stands for a fatty acyl radicle containing from 2 to 5 carbon atoms.

EDWIN A. ROBINSON,  
MAURICE J. KELLEY.